

J. H. WEEKS.  
PROCESS AND COMPOSITION FOR ELECTRICAL ETCHING.  
APPLICATION FILED JULY 8, 1916.

1,289,022.

Patented Dec. 24, 1918.

4 SHEETS—SHEET 1.



J. H. WEEKS.

PROCESS AND COMPOSITION FOR ELECTRICAL ETCHING.

APPLICATION FILED JULY 8, 1916.

1,289,022.

Patented Dec. 24, 1918.

4 SHEETS—SHEET 2.



Inventor  
Joseph H. Weeks  
Edward E. Blewett

Attorney

J. H. WEEKS.  
PROCESS AND COMPOSITION FOR ELECTRICAL ETCHING.  
APPLICATION FILED JULY 8, 1916.  
**1,289,022.** Patented Dec. 24, 1918.  
4 SHEETS—SHEET 3.



J. H. WEEKS,  
PROCESS AND COMPOSITION FOR ELECTRICAL ETCHING,  
APPLICATION FILED JULY 8, 1916.

1,289,022.

Patented Dec. 24, 1918.

4 SHEETS—SHEET 4.

Fig. 8.



Fig. 9.



Inventor  
Joseph H. Weeks  
By  
Edward E. Blawie  
Attorney

# UNITED STATES PATENT OFFICE.

JOSEPH HENRY WEEKS, OF RUTLEDGE, PENNSYLVANIA, ASSIGNOR TO JACKSON S. WEEKS, OF DELAWARE COUNTY, PENNSYLVANIA, AND RAYMOND M. WEEKS, OF PHILADELPHIA, PENNSYLVANIA, TRUSTEES.

## PROCESS AND COMPOSITION FOR ELECTRICAL ETCHING.

1,289,022.

Specification of Letters Patent.

Patented Dec. 24, 1918.

Application filed July 8, 1916. Serial No. 108,232.

*To all whom it may concern:*

Be it known that I, JOSEPH H. WEEKS, a citizen of the United States, residing at Rutledge, in the county of Delaware and State 5 of Pennsylvania, have invented certain new and useful Improvements in Processes and Compositions for Electrical Etching, of which the following is a specification, reference being had therein to the accompanying 10 drawing.

My invention relates to electrical etching and has for its object the provision of an improved process of and composition for electrical etching as hereinafter described.

15 The present invention is a continuation in part of my prior application, Serial No. 88,362, filed April 1, 1916, and is an improvement thereon in certain particulars, especially in regard to the composition of 20 the electrolyte.

Certain forms of apparatus made use of in carrying out my invention are illustrated in the accompanying drawings to which reference will be had in the description and in 25 which—

Figure 1 is a perspective view of the improved etching tank used in carrying out my invention.

Fig. 2 is a continuation of Fig. 1 showing 30 in perspective the driving mechanism.

Fig. 3 is a perspective view partly in section of the etching tank equipped with mechanically driven brushes for removing sludge from the cathodes.

35 Fig. 4 is a detail of the adjustable brush holder.

Fig. 5 is a perspective detail view showing the arrangement of the brush in this holder.

Fig. 6 is a detail of the brush rod adjust- 40 ment.

Fig. 7 is a detail of the link connection between the brush mechanism and the operating shaft.

Fig. 8 is a plan view of a tank with a 45 plate suspended therein, face down, and cathodes hung vertically upon wires along the sides and ends of the tank.

Fig. 9 is a longitudinal view of the same 50 partly in section, showing cams and slides for raising and lowering the plate in the solution while etching.

Referring to the drawings, and especially

to Figs. 1 and 2, 1 indicates an etching tank which may be of any suitable waterproof and insulating material, or other kind of 55 material rendered waterproof on the inside, such as wood coated on the inside with an insulating waterproof and chemical resisting material. The usual drain cock 2 is provided for the purpose of draining the tank 60 when necessary to change the solution or empty for repairs. Positioned within the tank around the four sides thereof so as to be immersed and substantially surround the electrolyte, are the cathodes 3 which may be 65 of any suitable conducting material but are preferably of carbon. As it is difficult to obtain and use, with economy, carbon plates of the dimensions and proportions desired, I find it expedient and advantageous to form 70 these cathodes of a number of carbon plates 4 held and protected by a frame 5. Electrical connection is made between the cathode plates 4 and a bus 6 by means of a plurality 75 of flexible conducting members 7 extending in parallel connection between the said cathode plates and bus bar. This bus bar 6 extends entirely around the outside of the etching tank near the top thereof, so as to afford the shortest possible connection between it and the cathode plates. Normally 80 resting upon the top of the tank and extending longitudinally thereof, is a continuous plate support 8 which rests upon the opposite ends of the tank 1 and is prevented 85 from coming in contact with the flexible connections 7 of the end cathode plates by the insulating blocks 9. Each of these blocks 9 is provided with transverse channels 10 in its lower surface to accommodate the conductors 7 and carries on its upper surface a pair of vertical guide rods 11 positioned 90 near the ends of the blocks so as to include the plate support 8 and prevent lateral displacement thereof during its up and down 95 movement.

In this up and down movement of the plate support 8 it is desirable that it be given a certain cycle of operation which I have found makes for better results and therefore 100 constitutes an important part of the process to which the present invention pertains. The driving and operating mechanism for producing the movement of the plate support

consists of a suitable prime mover such as the electric motor 12 mounted above the tank on the platform 13 supported on suitable wall brackets such as 14. The motor 12 is 5 connected through a reducing worm gear 15 to a countershaft 16 running parallel to the etching tanks, of which there may be any number, and carrying at its ends a pair of crank disks 16'. Each of these crank disks is 10 connected through a crank pin 17 and link 18 to a sliding shaft 19 bearing at its ends in slotted side brackets 20, which side brackets are arranged to permit the shaft 19 to move only up and down in a vertical plane 15 longitudinal of the tanks. Connection is made between the shaft 19 and plate support 8 by means of flexible connections 21. With this arrangement the comparatively slow rotary movement of the shaft 16 is transformed 20 into a variable vertical movement of the sliding shaft 19, due to the crank and pitman connection between them, shaft 19 having a higher speed midway of its extreme positions than at the extreme positions. 25 By adjusting the length of the flexible connections 21, I may obtain various degrees of lost motion between the plate support 8 and the shaft 19, whereby the continuous motion of the shaft 19 may be transformed into an 30 intermittent motion of the plate support, the cycle of which may be varied as regards the relative periods of rest and movements by adjustment of the length of the flexible connections 21. For example if the flexible connections 21 are so adjusted that when the 35 shaft 19 is at its highest point, the plate support 8 will swing a given distance above the insulating blocks 9, this distance will represent the limit of the amount of vertical 40 movement given to the plate support 8 and through it to any plates suspended therefrom in the electrolyte, any further movement that would otherwise be transmitted to it from the rod 19 being lost through the flexible 45 connection when the plate support comes to rest on the insulating blocks 9. Thus any plates carried by the support 8 will remain at rest in the solution during a certain portion of the cycle and be moved during the 50 remainder, the extent of movement and the relative duration of the rest and moving periods depending upon the amount of lost motion between the shaft 19 and support 8, while the duration of the complete cycle 55 would be determined by the speed at which the driving apparatus is operated. It is not desirable to have the plates move all the time, although this may be accomplished by adjusting the flexible connections 21 in a 60 manner that will be obvious. In any case the plates are of course immersed all the time. As a specific example of an adjustment to produce a given cycle, if the full stroke of the rod 19 is 11 inches and the connections 21 are adjusted to raise the plates 65

only 2 inches, the time of motion of the plates will be 2/11 of the whole cycle, while the period of rest will be 9/11 of the whole cycle.

During etching an occasional interruption 70 of the current is desirable, and in fact important, because it tends to keep the face of the anode (the plate being etched) clean, and assists in producing smoothness of etching. A plate to be so treated is indicated at 75 22 which is suspended from the support 8 by a suitable metallic hook 23 through which it receives current from the conducting support and which hook is so arranged that it may be lifted out of connection with the 80 member 8 to interrupt the flow of current to the plate 22. This lifting of the hook 23 with a resulting interruption of the current flow is effected periodically by means of a suitable flexible connection 24 connecting the 85 hook with the sliding rod 19 and so adjusted as to its length that the lost motion between the hook 23 and the rod 19 will be taken up before that of the support 8, thus causing the hook 23 to be raised slightly in 90 advance of the support 8 and held out of electrical contact with the support until it again comes to rest on the insulating blocks 9, when the connection 21 becomes slack and after that the connection 24, permitting the 95 hook 23 to again come to rest on the support 8 in electrical contact therewith. Thus, in the case of a plate connected as 22, it is not only periodically moved up and down in the electrolyte but has its supply of current 100 periodically cut off, the duration of either of which conditions may be varied by suitable adjustment of the flexible connections 21 and 24 in a manner which will be obvious. It is further to be noted that, if desired, the 105 plate 22 may be made to remain stationary during the whole cycle of movement of the rod 19 with only an interruption of the circuit once in each cycle. This of course could be effected by slackening the connections 21 110 sufficiently to allow the support 8 to remain stationary at all times.

For supplying current to the conductors 6 and 8, I provide a pair of looped bus bars 25 and 26, positive and negative respectively, running parallel to the several tanks and supported above and back of them on a suitable insulating wall support 27. From these bus bars connection is made through suitable protected flexible cables 28—29 and 115 30—31, to the conducting support 8 and bus 6, respectively. As a low voltage current is usually employed in apparatus of this kind and an even distribution of the volume of the current is essential, the arrangement of 120 certain connections must be such as to avoid any difference in the drop of potential at the different points of connection. It is to this end that the connection is made from opposite ends of the support 8 through separate 125 130

conductors 28 and 29 to individual positive bus bar members 25, and from opposite ends of the continuous bus 6 through separate conductors 30 and 31 to separate negative bus bar members 26. Where more than one tank is connected up at a time to the same dynamo, those connected nearest the dynamo to the bus members 25 and 26 will be subjected to a voltage slightly higher than the 10 farther tanks but with the arrangement of connection shown, this will not affect the even distribution of current as regards the individual tanks.

Where it is desired to surround the electrolyte on all four sides and bottom with the cathode members, a fifth cathode member is provided, which substantially covers the bottom of the tank and to which connection is made to all four edges thereof from the 20 four sides of the bus 6 by means of conducting members such as 32 passing through the side walls of the tank through suitable watertight insulating bushings 33.

When electrolytes are employed which 25 tend to form sludge or a coating on the cathodes, I provide mechanical means for disengaging the sludge and keeping the cathodes clean. A preferred form of this means is here illustrated in Figs. 3 to 7 inclusive, 30 and while for the sake of clearness I have not shown it combined with the arrangement of Figs. 1 and 2, it is to be understood, of course, that it is to be used in combination with the former arrangement of apparatus, 35 that is in association with a common tank. This cleaning arrangement consists generally of a set of brushes 34 arranged to be moved up and down across the inner faces of the cathodes by suitable reciprocating 40 mechanism such as the sliding shaft arrangement of Fig. 1 preferably identical therewith and which shall be so described.

Referring more in detail to the structure of the cleaning mechanism, the brushes 34 45 are connected to the side rods of the rectangular frame 35 through adjustable connecting devices 36 each comprising a frame or rod engaging portion 37 in the form of a collar and set screw and a brush engaging 50 portion 38 in the form of a C clamp having a pointed anchor stud 39 and clamping screws 40. With this novel form of connection between the brushes and the frame, the brushes may be set either to cause the edge 55 or the entire face to engage the cathode. To take up wear between the brushes and the cathodes, the rods forming the frame 35 are connected at each of the four sides through right and left threaded turn buckles 60 41. The brush carrying frame 35 is carried by a pair of forked rods 42 the tines of each fork connecting with the corners at opposite ends of the frame. The arm 43 of each forked rod carries a bifurcated member 65 44 in which is pivotally secured the lower

end of a connecting rod 45 having a U shaped head 46 open at the side and adapted to straddle the sliding shaft 19. The space between the arms of the U-shaped head is slightly tapered toward the open end so that 70 when the head is slid over the rod 19 the open end only will offer an appreciable resistance, the closed end fitting freely around the shaft. To secure connecting rod 46 against disengagement from the shaft 19, a 75 bolt or pin 47 is provided which extends across the open side through perforations 48 therein.

It will be seen that the forked members 42 are amply wide enough to permit free 80 operation of the plate support 8 and easy access to the different parts by the operator. When this cathode cleaning mechanism is used, it is preferable to omit the fifth or bottom cathode. 85

Figs. 8 and 9 show another form and arrangement of a tank and appurtenances for carrying out my process. In these figures, projections 50 on the sides of the tank carry a wire or rod 51 extending around the entire 90 upper part of the tank and having extension terminals connected to the negative terminal of the source of current.

My cathodes 52, consisting preferably of carbon rods provided with metal caps and 95 hooks at their upper ends, are hung from this wire. In Fig. 9 twelve of these cathodes are swung, but the number is immaterial, so long as their combined surface is greater than the surface of the anode or plate to be 100 etched. A liberal allowance in this respect is productive of good results. The anode or plate is shown at 53, suspended face down from a pair of rods 54, consisting of copper wire bent in a loop at each end, and connected at both ends to the positive terminal of the source of current, which is preferably a dynamo of low voltage, but may be any convenient and suitable source. 105

When a large quantity of solution is employed, the up and down motion of the anode can be dispensed with, but I consider it very desirable to gently move the anode at constantly recurring intervals as before described for Fig. 1. Mechanism for producing this motion of the plate is also provided in the form of apparatus shown in Figs. 8 and 9. I here show a shaft 55 beneath the tank, with its ends journaled in bearings secured thereto, provided with a pulley 56 at one end for attachment to any suitable driving means. Vertical slides 57 are provided on the ends of the tank which at their upper ends carry the wires or rods 54 and at their lower ends are slotted to slide up and down on the shaft, with roller bearings 58 resting upon the surface of rotary cams 59 on the shaft. As the shaft rotates, the cams 59 raise and lower the rollers 58 and the slides 57 to which they are attached, thereby raising 110 115 120 125 130

and lowering the wires 54, which play between guides 60 in the top of the tank.

In order to lessen the quantity of solution required in the tank, and also to draw the 5 heavy solution flowing from the anode plate directly to the base of the cathode or cathodes, I insert a filler or block shown in Figs. 8 and 9. This is geometrically shaped, preferably with triangular ends, sloping sides, 10 and its longitudinal ridge lying directly under the anode plate. It is made of acid-resistant material or wood or metal coated with the same and water-tight. This filler is shown at 61, in dotted lines, in Figs. 8 15 and 9.

I consider it novel and original with me to arrange the cathodes in the manner shown and described in the several figures so as to permit an even distribution of the current 20 in all parts of the bath. I have hitherto worked upon the generally accepted theory that the anode and cathode must face each other in parallelism so that the passage of current from one to the other through the 25 bath should be in lines as nearly normal to both surfaces as possible; but experience has shown me that this is unnecessary, provided that the points of sufficient surface and even distribution of current are taken care of.

30 For the solution or electrolyte in the tank, I may employ any one of a number of formulas, all well known to those skilled in the art. The regular electrotypers' formula so-called, consists of sulfate of copper dissolved in 35 water to make a solution testing 10 on the Baumé hydrometer, with sufficient sulfuric acid added to bring the hydrometer test to 15. This may be used, but I prefer certain formulas of my own, which I shall now state 40 and shall hereinafter claim as a part of my invention.

Solution No. 1: Dissolve calcium chlorid in water until the solution registers from 5 (with heavy Baumé hydrometer) to a point 45 of almost saturation. This solution can be used alone, but preferably I add an acid which may be nitric, hydrochloric, chromic, citric, or acetic. Other acids may be employed if desired. The proportion of acid 50 as well as the strength of calcium chlorid vary with the character of the work to be done. It is obvious that with the stronger acids, a smaller quantity thereof is required; and the stronger the calcium chlorid solution the larger the amount of acid which 55 may be employed. These acids increase the conductivity of the solution, which also varies with the strength of the chlorid solution. The acids also serve to keep the face 60 of the anode clean and bright.

Solution No. 2: This is made according to the foregoing formula, following the same remarks, but substituting sodium chlorid (common salt) in place of calcium chlorid.

65 Solution No. 3: This solution is made in

exactly the same way and according to the same directions as No. 1, but ammonium chlorid (salammoniac) is substituted for the calcium chlorid.

Solution No. 4: Dissolve sodium chlorid in 70 water until the solution tests 5 Baumé to saturation and combine in proper proportions a solution of ammonium chlorid of from 5 Baumé to saturation, adding any of the above named acids until the desired conductivity and effect on the anode are produced.

Solution No. 5: Ammonium chlorid in water to a strength testing from 5 Baumé (heavy 75 hydrometer) to saturation, to which is added from 5 per cent. to 100 per cent., of the volume of the former, a solution of perchlorid of iron containing an excess of acid; or a solution of neutral chlorid of iron used with the addition of an acid, as mentioned 80 in No. 1.

Solution No. 6: Sodium chlorid in water to a strength testing from 5 Baumé (heavy 85 hydrometer) to saturation, to which is added from 5 per cent. to 100 per cent., of 90 the volume of the former, of a solution of perchlorid of iron of about 42°, or chlorid of iron of equivalent strength, or the equivalent in dry chlorid of iron; with or without the addition of any of the acids mentioned 95 in No. 1.

Solution No. 7: Ammonium chlorid in water to a strength testing from 5 Baumé (heavy 100 hydrometer) to saturation, to which is added in any proportion desired a solution of sodium chlorid in water testing from 5 Baumé (heavy hydrometer) to saturation, and to the combined solutions is added from 5 per cent. to 100 per cent. of the volume of the former, solution of perchlorid of iron of 105 about 42° strength, or chlorid of iron of equivalent strength, or the equivalent in dry chlorid of iron; with or without the addition of any of the acids mentioned in No. 1.

As illustrations of solutions produced by 110 these formulas, I may note the following:

|                                     |       |        |     |
|-------------------------------------|-------|--------|-----|
| No. 1. Calcium chlorid in water to  |       |        |     |
| Baumé test 20                       | ----- | 1 gal. |     |
| Hydrochloric acid C. P.             | ----- | 1½ oz. | 115 |
| No. 2. Ammonium chlorid in water    |       |        |     |
| to Baumé test 20                    | ----- | 1 gal. |     |
| Sulfuric acid                       | ----- | 1 oz.  |     |
| No. 3. Sodium chlorid in water to   |       |        |     |
| Baumé test 20                       | ----- | 1 gal. | 120 |
| Sulfuric acid                       | ----- | 1¼ oz. |     |
| No. 4. Sodium chlorid in water test |       |        |     |
| 15                                  | ----- | ½ gal. |     |
| Ammonium chlorid in water           | ----- | ½ gal. | 125 |
| test 15                             | ----- | 1 oz.  |     |
| Hydrochloric acid                   | ----- |        |     |

Under certain conditions I find it of further advantage to lastly add to each of the solutions 5, 6 and 7 from ½ per cent. to 15 per cent., of the total preceding volume, 130

hydrochloric acid C. P., or the equivalent of hydrochloric acid of lesser strength. Other acids may also be employed as previously indicated.

5 Having thus described the apparatus and composition of the electrolytes, I shall now proceed with the steps in the operation.

The first step consists in producing the image on the plate by any of the photographic or transfer methods well known in the graphic arts.

The back of the plate is next coated with an insulating material, which may be chosen from a great variety, such as shellac dissolved in alcohol, a solution of asphaltum and paraffin, or almost any wax like substance, to which has been added a resin or asphaltum, or both.

The plate is then connected with the positive wire of a dynamo or battery and immersed in a suitable electrolyte, constituting the anode terminal therein. I have found it preferable and shall claim it as original, to maintain the plate horizontally in the electrolyte with the face (the side containing the image) downward, as hereinbefore described.

In line plates or what is known as line portions of combination plates, after a certain depth is attained, which is technically termed (in chemical etching), the "first bite" or "first etch," powdering with resinous or waxous powder is necessary. A variety of such powders have been in use, for a long time, by photo-engravers and others employing acid chemical means, to prevent the thinning of the lines by side etching, which would soon be followed by under cutting, or under etching of the lines, and if carried to an extreme degree, would necessarily take the line away entirely, or if only to a slight extent, would interfere with the duplication of the plate by electro-typing or stereotyping. To prevent this side etching and thinning of the lines after having obtained a certain depth, reinforcing the side of the lines must be done in four directions, whether the plate be etched electrically or chemically, and this I must therefore do in my electrical etching method, although I am able to obtain a greater depth before this becomes necessary than is possible in chemical etching. It may readily be seen that in very small spaces, such as between lines that are approximately one fiftieth of an inch apart, the powder entirely fills the opening and this receives no further etching after the first etching, so that the depth of the plate in such fine portions, therefore, depends entirely upon the etching. Herein I claim great superiority owing to the fact that my plate is 50 per cent. to 100 per cent. deeper than the old plates before the necessity for powdering arises.

65 After powdering more or less of a shoul-

der is produced, hence by getting my plate so much deeper in the first etching, the possibility of shoulders on the sides of the lines near the printing surface is entirely obviated. Shoulders, it may be added, increase 70 the difficulty of printing any plate.

It will be apparent to those skilled in the art that some sundry changes and modifications may be made in the apparatus, in the method and in such details as the formulas 75 of the electrolyte, etc. Thus, I may employ plates of various metals or substances, to be etched, and I may employ divers metals or other substances instead of carbon for the cathode, and in the apparatus mechanical 80 equivalents subserving the same function. For example adjustable rods engaging the sliding shaft 19 through elongated eyes or loops may be substituted for the adjustable 85 connections 21 and 24. These and all such other modifications that may be made without departing from the spirit of the invention and that fall within the scope of the appended claims, are contemplated by me.

In claiming my solution, I wish to call attention to the fact that I use the perchlorid of iron instead of the neutral iron and the subsequently added acid, as a matter of convenience, because the perchlorid of iron of commerce which is on sale in eastern cities of 95 the United States like Philadelphia, contains approximately the correct excess of acid. In some particular instances, on very delicate work, I have used the neutral iron combined with the sodium and ammonium 100 or either of them, where the resisting image was not thought to have sufficient strength to resist the stronger action of an acid solution, but such solutions would have no permanency. It is to be noted that the iron can be 105 omitted in etching for some of the metals, not including brass and copper, and with them it is to take care of the copper content that I use the iron especially. Thus, on other metals, a chlorid with an acid and 110 without the iron can be used and in some cases will work better. For this reason, and because the perchlorid which I employ contains an excess of acid, I desire to emphasize the fact that the acid is an important constituent for permanency in my electrolyte 115 and is present in the chlorid and may also be used without the iron. I shall therefore claim the solution with an acid and it is to be understood that such claim is generic to 120 those claims specifying perchlorid. It is to be also understood that while I have pointed out the usefulness of the iron in etching copper or an alloy containing copper, I do not wish to confine myself to such use, as 125 the perchlorid of iron is both convenient and efficacious with other metals, and can be used for example with steel, although I have not hitherto found it an essential ingredient in etching steel.

Having thus described my invention what I claim and desire to secure by Letters Patent is:

1. An electrolyte for electrolytic etching, 5 containing a solution of a chlorid, to which perchlorid of iron has been added.
2. An electrolyte for electrolytic etching composed of a solution of sodium chlorid to which has been added perchlorid of iron or 10 an equivalent as hereinbefore set forth.
3. An electrolyte for electrolytic etching composed of a solution of sodium chlorid to which has been added a quantity of perchlorid of iron and hydrochloric acid.
- 15 4. An electrolyte for the purposes described, composed of a solution of a chlorid of a member or a quasi-member of the alkaline group, to which has been added a quantity of perchlorid of iron and hydrochloric acid.
- 20 5. An electrolyte for electrolytic etching composed of a solution of sodium chlorid to which has been added perchlorid of iron or an equivalent, together with a quantity of 25 acid.
6. An electrolyte for electrolytic etching composed of a combined solution of ammonium chlorid and sodium chlorid to which has been added perchlorid of iron or an equivalent.
- 30 7. An electrolyte for electrolytic etching composed of a combined solution of ammonium chlorid and sodium chlorid to which has been added perchlorid of iron or an equivalent, together with a quantity of acid. 35
8. An electrolyte for electrolytic etching, consisting of a combined solution of ammonium chlorid and sodium chlorid to which has been added a quantity of acid. 40
9. An electrolyte for electrolytic etching composed of a solution of sodium chlorid to which has been added a quantity of perchlorid of iron and an acid. 45
10. An electrolyte for the purposes described composed of a solution of ammonium chlorid in water, combined with a solution of sodium chlorid in water, both testing approximately the same degreee Baume, to which has been added a quantity of perchlorid of iron and an acid. 50
11. An electrolyte for electrolytic etching composed of the chlorid of a member or quasi-member of the alkali group, in solution, to which has been added perchlorid of iron. 55
12. An electrolyte for electrolytic etching consisting of chlorid of sodium from 5 Baume to a point of saturation, with a small percentage of acid.

In testimony whereof I affix my signature. 60

JOSEPH HENRY WEEKS.